

Patented Dec. 25, 1923.

1,478,986

# UNITED STATES PATENT OFFICE.

JACQUE CYRUS MORRELL, OF NEW YORK, N. Y.

## PROCESS FOR THE MANUFACTURE OF ARTIFICIAL CHARCOAL.

No Drawing.

Application filed July 31, 1919. Serial No. 314,501.

To all whom it may concern:

Be it known that JACQUE C. MORRELL, a citizen of the United States, residing at New York, in the county of New York and 5 State of New York, has invented certain new and useful Improvements in Processes for the Manufacture of Artificial Charcoal, of which the following is a specification.

The present invention relates to the manufacture of artificial or synthetic charcoals such as are used for the adsorption and removal of impurities from air for respiration, and in various industrial and laboratory processes as the de-colorizing and purifying 15 agent.

It relates more particularly to the preparation of a mixture of carbon material and a binder which mixture is subsequently treated in the ordinary methods or in such 20 methods as are set out in my co-pending application Serial No. 284459 filed March 22, 1919, for artificial or synthetic charcoal and processes of producing the same.

Heretofore in preparing mixtures of carbon material and a binder, difficulty has been experienced in obtaining thorough distribution of the binder throughout the body of finely divided carbon material. This is readily recognized when it is considered that 30 the only binders suitable for such purposes are materials like pitch, which are either very viscous or very solid at ordinary temperatures.

In my co-pending application above referred to, I have described one method of accomplishing this distribution of the binder by suspending the binding material in the form of an emulsion or suspension in a very fluid medium, such as water. The present 40 invention has to do with a process of accomplishing a similar result in a different manner. The carbon material used in the present process is preferably carbon-black or lamp-black but such others materials as ground coke, coal, and wood-charcoal may be used. The binder that is to be used is pitch, or such materials as coal tar, bitumen and asphalt.

It will be readily realized that mixing such 50 binding materials with such carbon materials as are mentioned is very difficult, and since uniformity of distribution of the binder has a marked effect upon the porosity and uniformity of the charcoal, this question of properly incorporating the binder is vital.

The incorporation of the binder with the carbon material is accomplished in the present process by dissolving the binder in a suitable solvent, then intimately mixing 60 the carbon material and this solution, and subsequently distilling off from the mixture the solvent material, leaving deposited upon the individual particles of the carbon a film 65 of the binder. It may be remarked that such a process produces a material of which substantially each and every particle of the carbon material carries such a film of binder.

Suitable solvents for this purpose are benzene, solvent naphtha, toluene, xylene, carbon tetrachloride, low boiling point paraffine oil, or other suitable solvent whose boiling point is lower than the point at which the binding material begins to coke.

An example of one process involving the 75 present invention is as follows (parts being by weight):

About ten parts of the binder, such as soft coal tar pitch (made by mixing a heavy coal tar oil and hard pitch in suitable proportions) is dissolved in a solvent such as benzene, using from about twenty to about forty parts of the latter, depending on the carbon material to be used. Such carbon materials as carbon-black and lamp-black require a greater bulk of solution than heavier material.

The carbon-black (twenty or thirty parts) or other carbon material, is then thoroughly mixed with the solution.

The thin paste resulting from the above step is then placed in a suitable apparatus and the solvent distilled off and recovered, the temperature being controlled so as to remove only the solvent. The residue consists of the carbon material, the individual grains of which are coated with the film of the original binding material.

The product obtained by the above process can be readily compressed into a solid and subsequently treated in a fashion such as is described in my co-pending application above referred to. To accomplish the compression, this product is placed in a mold consisting of a sleeve, plunger and plug which is heated to about 90° C. and compressed with a pressure of 32,000-60,000 lbs. per square inch. Any substantial pressure, however, will suffice. The quality of the product improves with increase in pressure up to a certain point. 100 The function of molding under pressure is a very important one, determining to a large 105

extent the nature and quality of the finished product. The best types of charcoal possess a large degree of porosity and have supporting walls which are most dense. These are 5 the qualities which molding under pressure gives the finished product. Also, the pores and ducts of the carbon should be of the continuous or spongy type. If the residue is heated without first molding under pressure 10 a large proportion of the ducts are discontinuous and the product is friable because the walls are not sufficiently dense. In large scale work a rotary press, whose molds pass through a heated zone, may also be used. 15 The temperature to which it is necessary to heat is dependent upon the melting point of the pitch which in turn is dependent upon the percentage of oil in the mixture and the conditions can be controlled to allow 20 compression in the cold and the pressure may be varied within wide limits depending on the final product desired.

The crude charcoal from the press is crushed and ground to from 8 to 10 mesh or 25 any desired size. The grindings are utilized for regrinding to a powder after which they are recompressed without any other additions to produce charcoal. The ground material is introduced into a furnace and gradually brought to the decomposing temperature. Schedules of 4 hours at 850° C. then to 925° C. for one-half hour, and of 3 hours at 925° C. to 950° C. have proved satisfactory. 30

35 I have found that a final heat treatment following the above steps causes a marked improvement in the efficiency of the charcoal. This is true not only of synthetic charcoals but also of other charcoals as for 40 instance, standard cocoanut charcoal which showed an improvement of 50% in activity after this treatment. The apparent density of the charcoal after this treatment shows a pronounced lowering which, it is thought, is 45 caused by the internal oxidation by adsorbed air or the removal of hydrocarbons or both, by this heat treatment. Heating beyond a certain length of time in the first carbonization treatment causes little improvement in the charcoal. However, if the 50 charcoal is allowed to cool to about 250° C., removed from the furnace and cooled in the air to room temperature to prevent the adsorption of hydrocarbons by the charcoal, 55 upon a second heat treatment, the above described results take place. Since the walls of the furnace contain condensed hydrocarbons, the second heating is done in a different furnace (though if cleansed one furnace 60 will suffice). The conditions under which this heat treating process is carried on should be at about 850° C. to 950° C. for about 2 hours. A third heat treatment also shows beneficial results. Heating in the 65 presence of steam and other mild oxidizing

agents also produces beneficial results. This may be done by any well known method, for example, by introducing steam directly into the retort.

The carbon-black-binder mixture produced by the above process is a black powder which flows almost as readily as the original dry carbon-black, and advantage is taken of this fact in carrying out a modification of the above described method, which 70 modification also permits the accomplishing of a very desirable object.

In the distillation of crude tars and oils, such as coal and pine tars and petroleum oils, for the purpose of recovering the valuable low boiling components, much trouble is occasioned by the accumulation of the pitch upon the walls of the distillation apparatus. This pitch forms a thick lining 80 which acts as a heat insulator, incidentally 85 increasing fuel cost, and it is necessary at frequent intervals to interrupt the distillation process in order to remove this disturbing factor. The ordinary method of removal is to allow the apparatus to cool and 90 have the pitch chopped away by hand.

Since the carbon-black binder mixture produced as described above is pulverulent and has the property of flowing readily, it is proposed to utilize this property in preventing the accumulation of pitch upon the walls of the distillation apparatus or retort. 95 This may be readily done by adding to the crude tar or oil about to be distilled an amount of carbon-black or other carbon 100 material which corresponds to the amount of pitch which will be produced by distilling the tar or oil and distilling the mixture. If 105 will be found that the pitch and carbon-black may be readily raked out of the retort without the necessity of cooling the apparatus and without difficulty.

The pitch resulting from such distillation remains adsorbed upon the carbon-black or other carbon material and this mixture may 110 then be treated in the same manner as the mixture produced by the first process herein described.

The present invention, therefore, contemplates intimately mixing carbon-black or 115 other carbon material with a material which contains pitch and a low boiling solvent or a material which contains the constituents of such pitch and solvent and from which pitch and solvent may be produced by distillation.

By the term "carbon" as used in the claims, I propose to include pure carbon of natural or artificial origin or a mixture of natural or artificial origin which contains 125 a high percentage of carbon; also various charcoals of animal, vegetable or mineral origin.

It should be noted that the present invention is not limited to the exact details and 130

proportions herein given, as these may be varied and must be varied to some extent, depending upon the exact materials used, but is to be limited only by the appended 5 claims.

Claims:

1. In a process of making built-up structural adsorbent charcoal, mixing carbon in a finely divided condition with a solution in a low boiling solvent of a binder which chars on heating, distilling off the solvent, molding the residue under substantial pressure, charring the binding material therein and then activating by heating. 10
  2. In a process of making built-up structural adsorbent charcoal, mixing carbon in a finely divided condition with a solution in a low boiling solvent of a binder which chars on heating, distilling off the solvent, molding the residue under substantial pressure, comminuting the molded material and charring the binding material therein and then activating by heating. 15
  3. In a process of making built-up structural adsorbent charcoal, mixing carbon in a finely divided condition with a solution in a low boiling solvent of a binder which chars on heating, distilling off the solvent, molding the residue under substantial pressure, charring the binding material therein and then activating by heating and treatment with a mild oxidizing agent. 20
  4. In a process of making built-up structural adsorbent charcoal, mixing carbon in a finely divided condition with a solution in a low boiling solvent of a binder which chars on heating, distilling off the solvent, molding the residue under substantial pressure, comminuting the molded material and charring the binding material therein and then activating by heating and treatment with a mild oxidizing agent. 25
  5. In a process of making built-up structural adsorbent charcoal, mixing carbon in a finely divided condition with a solution in a low boiling solvent of a binder which chars on heating, distilling off the solvent, molding the residue under substantial pressure, charring the binding material therein and then activating by heating and steaming. 30
  6. In a process of making built-up structural adsorbent charcoal, mixing carbon in a finely divided condition with a solution in a low boiling solvent of a binder which chars on heating, distilling off the solvent, molding the residue under substantial pressure, comminuting the molded material and charring the binding material therein and then activating by heating and steaming. 35
- the binding material therein and then activating by heating and steaming. 40
7. In a process of making built-up structural adsorbent charcoal, mixing carbon in a finely divided condition with a solution in a low boiling solvent of tar pitch, distilling off the solvent, molding the residue under substantial pressure, charring the binding material therein and then activating by heating. 45
  8. In a process of making built-up structural adsorbent charcoal, mixing carbon in a finely divided condition with a solution in a low boiling solvent of tar pitch, distilling off the solvent, molding the residue under substantial pressure, comminuting the molded material and charring the binding material therein and then activating by heating. 50
  9. In a process of making built-up structural adsorbent charcoal, mixing carbon in a finely divided condition with a solution in a low boiling solvent of tar pitch, distilling off the solvent, molding the residue under substantial pressure, charring the binding material therein and then activating by heating and treatment with a mild oxidizing agent. 55
  10. In a process of making built-up structural adsorbent charcoal, mixing carbon in a finely divided condition with a solution in a low boiling solvent of coal tar pitch, distilling off the solvent, molding the residue under substantial pressure, comminuting the molded material and charring the binding material therein and then activating by heating and treatment with a mild oxidizing agent. 60
  11. In a process of making built-up structural adsorbent charcoal, mixing carbon in a finely divided condition with a solution in a low boiling solvent of coal tar pitch, distilling off the solvent, molding the residue under substantial pressure, charring the binding material therein and then activating by heating and steaming. 65
  12. In a process of making built-up structural adsorbent charcoal, mixing carbon in a finely divided condition with a solution in a low boiling solvent of coal tar pitch, distilling off the solvent, molding the residue under substantial pressure, comminuting the molded material and charring the binding material therein and then activating by heating and steaming. 70

In testimony whereof I affix my signature.

JAC CYRUS MORRELL.